

## UNITED STATES PATENT OFFICE

CHARLES E. BURKE AND WALTER E. LAWSON, OF WILMINGTON, DELAWARE, ASSIGNORS  
TO E. I. DU PONT DE NEMOURS & COMPANY, OF WILMINGTON, DELAWARE, A COR-  
PORATION OF DELAWARE

## WATERPROOFING COMPOSITION AND ARTICLES TREATED THEREWITH

No Drawing.

Application filed July 9, 1928. Serial No. 291,480.

This invention relates to the art of waterproofing compositions, and more particularly to the waterproofing of paper and articles made therefrom, such as shotgun shells.

5 Present methods of waterproofing shotgun shells usually involve the use of paper treated with paraffin, vegetable oils, or pyroxylin, or combinations of these materials, as impregnating or coating agents. It has 10 been found, however, that shells so treated have not possessed the desired characteristics of being waterproof and sufficiently rigid to hold their shape and at the same time preserve their elasticity.

15 It is therefore an object of this invention to improve the waterproofing of paper and articles treated therewith.

It is another object of this invention to produce a stiffer and more uniform shell, so 20 that better patterns are secured and more uniform velocity is obtained, and to produce a shell having an improved appearance.

It is a further object of this invention to improve the waterproofing and stiffening of 25 a shotgun shell without unduly sacrificing its elasticity.

It is also an object of this invention to make shells more resistant to abrasion, which is caused by the long continued tumbling often 30 encountered when shells are carried loose in a hunting jacket, so they will retain their close shooting qualities.

We have found that these objects can be accomplished by treating paper or articles 35 made therefrom, such as shotgun shells, with solutions containing a polymerizable substituted ethylene. An example of such a polymerizable substituted ethylene is styrene which can be dissolved in a suitable solvent 40 (with or without a softener, and with or without coloring matter), applied to the shell, and polymerized by standing, or (more rapidly) by heating to form a hard, resistant, and waterproof surface.

45 We have found that these objects can be

accomplished by coating or impregnating paper or articles made therefrom with the compositions set forth below in the form of spraying or dipping lacquers. It should be understood that these compositions are merely set forth by way of illustration and not as a limitation.

## Example 1

|                                                                   | Parts by weight |
|-------------------------------------------------------------------|-----------------|
| Meta styrene                                                      | 18 55           |
| Tricrésyl phosphate                                               | 3.6             |
| Solvent—Ethyl acetate 20; butyl acetate 30; toluene 30; xylene 20 | 100             |

Used as a spraying lacquer over paraffin impregnated shells, one coat increased the time limit for total immersion in water without swelling or opening of crimp from two hours to seven hours. Used as a dipping lacquer, two coats increased the time limit to eight hours.

## Example 2

|                                                                                              | Parts by weight |
|----------------------------------------------------------------------------------------------|-----------------|
| Vinyl chloride, alpha polymer                                                                | 18 70           |
| Blown China wood oil (containing 0.5 pts. cobalt linoleate drier)                            | 18.5            |
| Solvent—Acetone 36; ethyl acetate 36; butyl acetate 45; chlorobenzene 45; hexalin acetate 20 | 182 75          |

This composition gave results similar to those in Example 1.

## Example 3

|                                                                               | Parts by weight |
|-------------------------------------------------------------------------------|-----------------|
| Polymerized vinyl chloroacetate                                               | 25              |
| Solvent—Ethyl acetate 40; butyl acetate 35; acetone 15; cellosolve acetate 10 | 100 90          |

Used as a dipping lacquer, two coats on shotgun shells increased the time limit for total immersion without swelling or crimp loosening from two hours for the untreated shells to from five to five and one-half hours for the treated shells.

*Example 4*

|                                                                            | Parts by weight |
|----------------------------------------------------------------------------|-----------------|
| Vinyl chloride, acetone soluble polymer                                    | 11              |
| Polymerized vinyl acetate                                                  | 11              |
| 8 Solvent—Acetone 20; ethyl acetate 20; butyl acetate 30; chlorobenzene 30 | 100             |

Used as a dipping lacquer, two coats increased the time limit to seven hours.

10

*Example 5*

Instead of using a mixture of two vinyl compounds polymerized separately, a product obtained by polymerization in mutual contact may be used, as in the following case:

|                                       | Parts by weight |
|---------------------------------------|-----------------|
| Vinyl chloride-vinyl acetate polymer  | 37              |
| Solvent—acetone 25; ethyl acetate 25; |                 |
| 20 butyl acetate 20; toluene 30       | 100             |

This mixture, being of greater viscosity than any of the preceding lacquers, gave exceptionally high protection. Shotgun shells were protected for 20 to 24 hours and even longer without any change in their appearance.

Although the examples given are limited to meta styrene and vinyl esters, many other compositions are useful for this purpose, such as polymers of other vinyl esters, especially the esters of higher fatty acids and polymerized vinyl ethers; polymers of allylene compounds; homologues of meta styrene, such as polymers of ethyl styrene and para-methyl styrene; and polymers of other highly unsaturated hydrocarbons.

We have found it desirable to modify meta styrene and its homologues, such as meta paramethyl styrene and other substitution products, to soften them and render them less brittle, suitable softeners including dibutyl phthalate, tricresyl phosphate and butyl stearate.

45 We have also found it desirable to modify polymerized vinyl chloride, by treating with suitable softeners, such as dibutyl phthalate or glyceryl dibenzyl ether, by mixing with drying oils, such as China wood, linseed, and perilla oils, or by adding other compatible vinyl derivatives, such as vinyl acetate.

These compounds may be incorporated in spraying or dipping lacquers and used as coating compositions on loaded shells, or may be employed for the impregnation of shells previous to loading. If desired, the impregnated shells, previous to loading, may be subjected to a baking process to increase their water resistance. For example, the water resistance of shells treated with polymerized vinyl chloracetate is markedly increased by baking at 65° C. for two hours, or at higher temperatures for correspondingly shorter periods of time. If the loaded shells are of the ordinary paraffin impregnated type, it is usually advisable to wash the shells with a

solvent for paraffin such as benzene or gasoline, or to subject them to a moderate buffing treatment.

Although we have stressed herein the use of our coating composition for waterproofing shotgun shells, it is equally useful for waterproofing or moisture-proofing paper for other purposes.

As many apparently widely different embodiments of this invention may be made without departing from the spirit thereof, it is to be understood that we do not limit ourselves to the foregoing examples or description, except as indicated in the following patent claims.

We claim:

1. A shotgun shell treated with a composition containing meta styrene.

2. A shotgun shell coated with a composition containing meta styrene.

3. A shotgun shell coated with a waterproofing composition containing about 18 parts by weight of meta styrene, about 3.6 parts by weight of tricresyl phosphate, and about 100 parts by weight of solvent.

In testimony whereof we affix our signatures.

CHARLES E. BURKE.  
WALTER E. LAWSON.

95

100

105

110

115

120

125

130